

Jan. 26, 1937.

E. C. BAIN ET AL

2,068,785

METHOD OF MANUFACTURING LOW CARBON STEEL

Filed Nov. 20, 1933



Inventors  
Edgar C. Bain and  
Herbert Gruber

BY *Herbert Gruber*

ATTORNEYS

## UNITED STATES PATENT OFFICE

2,068,785

## METHOD OF MANUFACTURING LOW CARBON STEEL

Edgar C. Bain and Herbert Gruber, Hanau-on-the-Main, Germany, assignors, by mesne assignments, to United States Steel Corporation, a corporation of New Jersey

Application November 20, 1933, Serial No. 698,922

7 Claims. (Cl. 75—12)

- This invention relates to metallurgy and more particularly to steel metallurgy and to methods of decarburizing molten steel baths. Still more particularly the present invention relates to a method of decarburizing iron and steel alloys containing one or more of the strong carbide forming elements, chromium, vanadium, tantalum, manganese, columbium, uranium, titanium and the like.
- 10 One of the objects of the present invention is to provide an efficient method for decarburizing iron and steel alloys containing one or more of the strong carbide forming elements.
- Another object of the present invention is to provide a method of decarburizing iron and steel baths to a relatively low carbon content without consequent oxidation of the strong carbide forming elements or other metal constituents of the said alloy.
- 20 Still another object of the present invention is to provide a method for manufacturing low carbon, iron and steel alloys particularly those alloys containing chromium without oxidizing the said alloy or constituents thereof.
- 25 Other objects and advantages will be apparent as the invention is more fully disclosed.

In accordance with the objects of the present invention, we have devised a method of decarburizing molten iron and steel alloys comprising a succession of treatment steps applied to the molten alloy, each step employing a controlled atmosphere operating to remove carbon and oxygen from the molten metal bath. As a result thereof, we obtain as a final product an extremely low carbon alloy which is substantially free from metal oxide compounds, the said process being highly practical and economical in operation as compared to methods heretofore devised. As a specific embodiment of the practice of the present invention but not as a limitation thereof we will describe the method as it is applied to the manufacture of low carbon, oxide free iron and steel alloys containing a proportion of the strong carbide forming element chromium. The same sequence of steps comprising the present method as is applicable to chromium-containing iron and steel alloys will be in general equally as applicable to other iron and steel alloys with slight modifications within each step thereof to accommodate the method to each specific alloy.

Before further disclosing the present invention, reference should be made to the accompanying drawing, wherein—

The figure is a sectional side elevation of a furnace useful in the practice of the present

invention with the associated apparatus used therewith schematically indicated.

The method of the present invention substantially comprises a series of successively applied steps or operations, each operation employing a different and controlled atmosphere. The process involves (1) the maintenance of the metal bath in a molten state throughout the interval of application of the series of treatment steps thereto preferably by means of induced electrical currents, the said induction heating means being designed to give relatively high turbulence to the molten metal of the bath so that all parts of the bath are recurrently brought to the surface for exposure to the controlled atmosphere over the said surface; (2) the maintenance over the surface of the metal bath of a succession of controlled atmospheres whereby the progressive removal of carbon from the bath to the low percentage desired is effected; (3) the addition to the metal bath of a carbon-reducible oxidizing material to facilitate the removal of carbon from the bath; (4) the application thereto of a final atmosphere effective to remove the final residues of carbon and oxygen from the bath; and (5) the degasification of the metal bath before casting and solidification.

As the broad idea is applied to iron and steel alloys containing chromium, the steps of the method of the present invention comprises—

(1) A treatment of the molten metal bath in an air atmosphere wherein the carbon content is oxidized to a low level;

(2) A treatment of the molten metal bath in a reducing gas atmosphere in the presence of an oxidizing material wherein the carbon content is still further reduced;

(3) A treatment of the molten metal bath in substantially pure dry hydrogen wherein the carbon content is reduced to a desired low percentage; and

(4) A degasification step before the decarburized and deoxidized molten metal bath is removed from the furnace.

As the broadly defined steps of the present invention is applied to iron and steel alloys containing chromium, the said alloy is heated to fusion and placed in an induction furnace "A" of the general type shown in the figure of the drawing. In this type furnace, the metal bath is held in refractory lined crucible 2 about which is positioned the transformer core 3 including a plurality of induction coils 4 so positioned about the crucible 2 and electrically connected together as to produce in metal bath 1 a

high turbulence or violent agitation. As the specific furnace structure or induction heating means forms no part of the present invention it need not be further described.

- 5 Over the top of the furnace "A", we place cover "B" which is hermetically sealed to furnace "A". Furnace cover "B" is provided with inlet and outlet pipes 5 and 6 respectively, inlet pipe 5 being provided with a plurality of connecting leader 10 pipes 1, 8, 9 and 10 having valves 11, 12, 13 and 14, which pipes 1, 8, 9 and 10 connect respectively to the atmosphere and to gas storage tanks 15, 16 and 17. Outlet pipe 6 is connected through valve 18 to evacuating means 19.
- 15 In accordance with the present invention, the molten metal bath 1 comprised of iron or steel and containing chromium is first subjected to decarburization in an air atmosphere at atmospheric pressures which is obtained by opening valve 11 (valves 12, 13 and 14 remaining closed). A high carbon alloy will rapidly oxidize in air at atmospheric pressures but oxidation of the carbon content thereof will proceed only to the extent where the residual carbon of the alloy 20 approximates an equilibrium percentage which varies somewhat with respect to the temperature employed and the amount of chromium present in the alloy. The chromium present thereafter 25 will tend to oxidize. It is advisable, therefore, to terminate this oxidation step before appreciable amounts of chromium have become oxidized. The precise time of termination of this step may be readily ascertained by one skilled in the art by appropriate analysis of the gas effluent from the furnace or by observing the appearance of oxide on the bath surface. The evacuating means 19 is not employed in this step as a 30 means to maintain a reduced pressure in furnace "A" but is utilized as a means for maintaining a circulation of air at atmospheric pressures through the furnace. Due to the high turbulence in metal bath 1, the rate of reaction of the oxidation process is relatively high and a strong free flow of air through furnace "A" is required.
- 35 45 The low limit of carbon content of the chromium alloy obtainable by the practice of this step approximates .30% although dependent in part upon the chromium content of the alloy.
- 50 With higher chromium, the lower limit of carbon will generally be higher.
- In the second step of the present invention, we add to the metal bath through opening 20 provided with sealable cover 21, a proportion of 55 carbon-reducible oxidizing material which is preferably comprised of one or more of the metal oxides of iron, chromium, nickel or oxidized ores thereof which are substantially free from associated silica and gangue impurities. We may, however, add to the said oxidizing material a proportion of heretofore known "slagging" materials such as fluorspar which will facilitate contacting the said oxidizing material with the molten metal bath. Thereafter, valve 11 is closed and the 60 molten metal bath is subjected to a combined decarburizing and deoxidation step at atmospheric pressures utilizing as a controlled atmosphere a hydrogenous reducing gas. In this step, valve 12 is opened, thereby permitting a hydrogenous reducing gas such as water gas, coal gas 65 mixed with blast furnace gas and the like to circulate into furnace 1 in sufficient volume to substantially maintain the pressure therein at atmospheric pressures, evacuating means 18 being utilized to maintain a strong free flow of such

gas through the said furnace "A". Alternatively, the gas can be supplied under high pressure sufficient to move it through the furnace in a strong free flow at atmospheric pressure or a little higher.

5 Preferably, the reducing gas employed is comprised of hydrogen, carbon monoxide and nitrogen with or without additions thereto of hydrocarbon gases or vapors. The hydrogen and nitrogen content of the reducing gas is preferably in 10 such relative proportions as to be substantially nonexplosive in nature. The carbon monoxide content may vary widely from about 10 to about 40 per cent (by volume) of the hydrogen-nitrogen admixture and the proportion of hydrocarbon 15 vapors or gases added thereto may vary with respect to the specific hydrocarbon gas or vapor employed, the temperature of the bath and with respect to the composition of the bath. This proportion of hydrocarbon gas or vapor should be 20 below that amount at which deleterious carbon absorption in the metal bath will occur. It is desirable that the reducing gas be substantially free from oxidizing gases such as water vapor, 25 carbon dioxide and the like as well as of hydrogen compounds of sulfur and phosphorus. Otherwise water vapor or carbon dioxide can be compensated by adding an excess of hydrocarbon vapor.

30 In general, and with most chromium alloys, it is advisable during the circulation of this reducing gas to increase the temperature of the bath to temperatures above the melting point of the alloy but not in excess of 2100° C., to reduce 35 the absorption of carbon by the bath from the gaseous atmosphere.

This decarburizing and deoxidizing step is continued for a determined time interval which is productive of the result desired. The specific 40 time interval will vary with different alloys and with the degree of deoxidation required. The carbon content of the bath by the practice of this step may be reduced as low as .08 per cent but this precise per cent is also dependent upon 45 the specific chromium content of the alloy.

The next step, of the present invention, is the 50 final decarburizing step and consists in gradually cutting off the volume of the hydrogenous reducing gas of step 3 and in gradually adding thereto substantially pure dry hydrogen until the 55 gas flowing into the furnace consists of substantially pure dry hydrogen. The temperature of the bath should be maintained at the higher temperatures of the preceding step during at least the first or initial stages of this hydrogen decarburizing step and thereafter may be dropped to any lower temperatures at which the bath will remain freely fluid. If the chromium content of the bath exceeds 50-60% or if it be desirable to carry out the process at as low a temperature as possible, a certain amount of hydrocarbon may be added to the pure dry hydrogen the amount of carbon in form of hydrocarbon not exceeding 30 to 50 grams per cubic meter of 60 hydrogen.

This step of the process is maintained for a 65 time interval required to bring the carbon content of the alloy to as low a per cent as desired or to a low percentage approximating .01 per cent. The precise time interval of treatment will vary 70 with respect to the alloy composition, chromium content and total carbon to be removed (mass of alloy treated). The progress of the step may be followed by analysis of the gas effluent from 75

furnace 1 or by any other convenient manner as desired.

When the desired low limit of carbon has been obtained in the metal bath 1, the hydrogen in furnace "A" may be displaced by substantially pure dry nitrogen from source 17 by closing valve 13 and opening valve 14. The molten metal bath 1 may thereafter be degasified by shutting off the nitrogen flow and evacuating the furnace "A" to a relatively low pressure.

Alternatively, the hydrogen flow may be terminated and the molten bath exposed to the air for a time interval to obtain substantial elimination of excess hydrogen contained therein, in which case it is desirable to add to the molten bath a small proportion of deoxidizing agent such as metallic silicon and the like before casting.

The molten metal thus treated may be poured from furnace "A" into a ladle, degasified by the addition thereto of gas scavenging elements zirconium, titanium, aluminum, silicon and the like and may be thereafter cast into ingot or other desired shapes. Where a high carbon ferro-chromium alloy is decarburized by this process, it may be added directly to a low carbon steel bath to form a desired chromium steel alloy.

From the above description of the method of the present invention, it is apparent that it is adapted to wide use and application in the production of low carbon iron and steel alloys. While as a specific embodiment we have described the application of the method of the present invention to chromium-containing iron and steel alloys, it is apparent that we are not to be limited thereby, as the same sequence of steps of the method described is equally as well applicable to other iron and steel alloys. The only modifications of the process described that is necessary for such other alloys are modifications in the time, temperature and gas compositions in each specific step to adapt the step to produce the desired result of the method as it has herein been described with respect to chromium alloys.

In view thereof, all such modifications and adaptations of the present invention are contemplated as may fall within the scope of the following claims.

What we claim is:

1. The method of decarburizing, deoxidizing and degasifying molten iron and steel alloys which comprises melting the said alloy and imparting thereto turbulent stirring to recurrently bring all parts of the bath to the surface and then applying to the said surface a succession of

atmospheres while maintaining the bath molten and turbulently stirred, including first an oxidizing atmosphere whereby the carbon is removed from the bath to a relatively low percentage without excessive oxidation of the metal constituents of the bath; second, a reducing gas atmosphere composed principally of hydrogen whereby the carbon content of the bath is further reduced to a still lower percentage while preventing substantial oxidation of the metal constituents of the bath; thirdly an atmosphere of substantially pure dry hydrogen having a relatively low water vapor content whereby the final carbon content is reduced to an extremely low percentage and the oxygen content of the bath is substantially eliminated; and fourthly, the bath is subjected to heating with turbulent stirring under reduced pressure to remove gases therefrom, the time interval of application of each successive step and the temperature of the molten metal being varied to promote the desired reaction.

2. In the method of claim 1, the addition of carbon reducible solid oxidizing agents to the molten metal bath prior to the said second step

25

3. In the method of claim 1, the addition to the molten metal bath prior to the application of the second atmosphere thereto of a proportion of solid carbon reducible oxidizing agents and a proportion of fluxing materials facilitating the 30 contacting of the said agent with the metal bath.

4. In the method of claim 1, the said succession of atmospheres being supplied in a strong free flow over the surface of the bath.

5. In the method of claim 1, the step of increasing the temperature of the bath to temperatures up to about 2100° C. during the decarburizing in the reducing gas atmosphere and during at least the early stages of decarburizing and deoxidizing in substantially pure dry hydrogen, 40 thereafter lowering the temperature of the bath to temperatures at which the bath remains freely fluid.

6. In the method of claim 1, the use of substantially pure dry nitrogen as a flush gas at the 45 conclusion of the hydrogen treating and prior to the final degasification step.

7. In the method of claim 1, the steps of melting and turbulently stirring the molten metal by induced electric currents, said currents inducing 50 vertical rotation of the bath at a plurality of points as well as horizontal rotatory circulation.

HERBERT GRUBER.  
EDGAR C. BAIN.